

## UNITED STATES PATENT OFFICE

2,261,862

## LUBRICANT

William A. Whittier, Kenilworth, Ill., assignor to  
The Pure Oil Company, Chicago, Ill., a corpora-  
tion of Ohio

No Drawing. Application December 18, 1937,  
Serial No. 180,487

19 Claims. (Cl. 252—58)

This invention relates to lubricants and to the method of preparing and of using the same, and is more particularly concerned with lubricants having extreme pressure characteristics.

It is well known that mineral lubricating oils can be improved by adding thereto halogenated aromatic hydrocarbons and compounds, in which hydrogen in the aromatic nucleus is substituted by chlorine. Halogenated aliphatic hydrocarbons and compounds in general have been found to be unsatisfactory because such compounds hydrolyze readily in contact with water forming acid which corrodes the metal surfaces.

I have discovered that where halogen is linked to aliphatic carbon, which is protected on both ends by a non-acidic, stable aromatic or other carbocyclic nuclei, the resulting compounds are not only not corrosive but are more active than the halogenated aromatics. Such compounds have the ability to impart to mineral lubricating oils, increased oiliness, film strength, and extreme pressure characteristics.

The compounds which I have discovered to be suitable are those of the type



in which R and R' are non-acidic, stable aromatic or other carbocyclic nuclei, either the same or different, C represents an aliphatic radical either saturated or unsaturated having any number (n) of carbon atoms in excess of one carbon, and Ha represents a halogen united to one or more aliphatic straight chain carbon atoms which are linked between the carbocyclic nuclei.

Examples of compounds which are suitable for use are symmetrical diphenyl ethane (diphenyl), symmetrical diphenyl ethylene, symmetrical diphenyl acetylene, symmetrical diphenyl butane, symmetrical diphenyl propane, symmetrical diphenyl butadiene, 1 phenyl 3-naphthyl propane, 1-naphthyl 4-phenyl butene-2, symmetrical di-naphthyl propane, 1-xenyl 4-phenyl butane, 1-naphthyl 3-xenyl propane, 1-4 dixenyl butane, 1-4 ditolyl butadiene, symmetrical diphenyl diethyl ether, 1-phenyl 6-naphthyl dipropyl ether, and symmetrical diphenyl ethylene ether, in which halogen is united to one or more aliphatic carbon atoms linked between the aromatic nuclei. The halogen may be added directly to the carbon in those compounds which are unsaturated or may replace the hydrogen in those compounds which are saturated. In the case of unsaturated compounds, halogen may be linked to

the carbon by direct addition, and by substitution of the hydrogen. Generally speaking, the greater the number of chlorine atoms linked to the carbon, the greater the activity of the compound and the greater is its effectiveness.

To illustrate graphically the nature of the compounds with which this invention is concerned,



By using 3 molecules of chlorine the hydrogen can be replaced and 2 chlorine atoms attached to each carbon thereby obtaining tetrachlor dibenzyl. This type of reaction is relatively simple and well understood.

The halogenated compounds may be used in connection with straight mineral lubricating oils or in connection with oils which have been blended with other reagents to improve the lubricating characteristics thereof. For example, I have found that when small quantities of halogenated compounds of the nature of those above described are incorporated in a blend of mineral lubricating oil with a sulfurized and phosphorized fatty oil base such as that disclosed in the application of Whittier et al., Ser. No. 55,200, the extreme pressure characteristics of such lubricants can be materially improved. A number of tests have been made on straight lubricants blended with halogenated compounds of the nature of those above set forth and on lubricants blended with sulfurized and phosphorized base together with halogenated compounds, and the results given in the table below. In these tests the straight mineral oil used was a blend in the proportions of 1:1 of two mineral lubricating oils of the following characteristics:

Table I

|                              | Oil No. 1 | Oil No. 2 |
|------------------------------|-----------|-----------|
| A. P. I. gravity             | 21.5-23   | 17-19     |
| Flash, °F.                   | 345-365   | 510-520   |
| Fire, °F.                    | 385-405   | 590-600   |
| Vis. at 130° F. (Say. Univ.) | 98-102    | 1750-2100 |
| Vis. at 210° F. (Say. Univ.) | 43-45     | 150-165   |
| Pour point, °F.              | -20       | 25        |
| Color N. P. A.               | 2-3       | 8         |

In those tests in which an oil blended with sulfurized-phosphorized base was used, the lubri-

cating oil, before addition of the base, had the following characteristics:

Table II

|                                   |         |
|-----------------------------------|---------|
| A. P. I. gravity-----             | 18-20   |
| Flash, °F-----                    | 380-400 |
| Fire, °F-----                     | 430-450 |
| Vis. at 130° F. (Say. Univ.)----- | 460-500 |
| Vis. at 210° F. (Say Univ.)-----  | 90-95   |
| Pour point, °F-----               | 0       |

This oil was blended with sulfurized-phosphorized base in the proportion of 82% of oil to 18% of base.

The sulfurized-phosphorized base was made in

kettle. When this temperature had been reached, 44 pounds of phosphorous sesqui-sulfide was added slowly over a period of  $\frac{1}{2}$  hour of continuous agitation. The steam was again turned on at such times as was necessary to maintain the temperature at 220° to 230° F. After the addition of phosphorous, agitation was continued for a period of approximately 5 hours while the temperature was maintained at 220° to 230° F. At the end of this period the contents of the kettle were immediately cooled to 130° F. by circulation through the exteriorly located cooling coils and pumped to storage.

The following is a table of the results obtained:

Table III

| Halogenated compound added               | Percent added | Oil used for blend               | S. A. E. test     |                 |
|------------------------------------------|---------------|----------------------------------|-------------------|-----------------|
|                                          |               |                                  | 1,000<br>R. P. M. | 750<br>R. P. M. |
| Trichlor dibenzyl-----                   | 5             | Sul-phos. base blend-----        | Pounds            | Pounds          |
| Do-----                                  | 8             | Plain mineral oil lubricant----- | 90                | -----           |
| Tetrachlor dibenzyl-----                 | 3             | Sul-phos. base blend-----        | 50                | -----           |
| Do-----                                  | 2             | do-----                          | 310               | -----           |
| Do-----                                  | 4             | do-----                          | 550               | -----           |
| Do-----                                  | 4             | do-----                          | 310               | -----           |
| Do-----                                  | 5             | do-----                          | 400               | -----           |
| Do-----                                  | 7             | do-----                          | 400               | -----           |
| Do-----                                  | 4             | do-----                          | 320               | -----           |
| Do-----                                  | 5             | do-----                          | 430               | -----           |
| Do-----                                  | 7             | do-----                          | 390               | -----           |
| Do-----                                  | 4             | do-----                          | 350               | -----           |
| Do-----                                  | 5             | do-----                          | 340               | -----           |
| Do-----                                  | 6             | do-----                          | 430               | -----           |
| Do-----                                  | 7             | do-----                          | 560               | -----           |
| Do-----                                  | 8             | do-----                          | 560               | -----           |
| Do-----                                  | 8             | Plain mineral oil lubricant----- | 340               | -----           |
| Hexa chlor sym. diphenyl butane-----     | 2             | Sul-phos. base blend-----        | 230               | -----           |
| Do-----                                  | 3             | do-----                          | 550               | -----           |
| Do-----                                  | 4             | do-----                          | 560               | -----           |
| Do-----                                  | 5             | do-----                          | 550               | -----           |
| Penta chlor sym. diphenyl pentane-----   | 3             | do-----                          | 330               | -----           |
| Do-----                                  | 8             | Plain mineral oil lubricant----- | 120               | -----           |
| Do-----                                  | 1             | Sul-phos. base blend-----        | 170               | -----           |
| Do-----                                  | 2             | do-----                          | 550               | -----           |
| Do-----                                  | 3             | do-----                          | 550               | -----           |
| Do-----                                  | 4             | do-----                          | 410               | -----           |
| Do-----                                  | 5             | do-----                          | 430               | -----           |
| Do-----                                  | 1.25          | do-----                          | 370               | -----           |
| Do-----                                  | 1.5           | do-----                          | 400               | -----           |
| Do-----                                  | 1.75          | do-----                          | 435               | -----           |
| Hexa chlor sym. diphenyl nonane-----     | 2             | do-----                          | 550               | -----           |
| Octa chlor sym. diphenyl nonadecane----- | 2             | do-----                          | 380               | -----           |

the following manner: A homogeneous mixture of 570 pounds of Gulf Coast pale oil having a Saybolt Universal viscosity of 200 seconds and a pour point of -20° to -25° F. and 55 pounds of sulfur chloride was prepared in a cold state. This mixture was added to 9,581 pounds of prime lard oil contained in an enclosed steam jacketed kettle. The mixture was heated to 275° F. while being vigorously agitated. At this point the steam was shut off and 814 pounds of flowers of sulfur were sifted into the contents of the kettle over a period of approximately 2 hours. The contents of the kettle were vigorously agitated during this entire period. At the end of the 2-hour period the temperature had dropped to 265° F. The steam was again turned on and the contents of the kettle heated to approximately 300° F. when the steam was turned off. Agitation was continued for a period of approximately 7½ hours after the addition of the sulfur. During this period the temperature rose from 300° to 344° F. during the first 3 hours indicating that an exothermic reaction was taking place. The temperature during the 7½-hour period was not permitted to drop below 320° to 330° F. and it was found that it was unnecessary to use any further heat to maintain this temperature after the mixture had been initially heated to 300° F.

The sulfurized material was then cooled to a temperature of 220° to 230° F. by circulating the material through cooling coils and back to the

50 The tests were made on the SAE extreme pressure testing machine which is used in the automotive industry to determine the suitability of extreme pressure lubricants. The maximum load that can be measured on the machine with safety is between 550 and 570 pounds.

55 As shown above, the sulfurized-phosphorized lubricant, without addition of the halogen compound, withstood a load of only 90 pounds. A comparative test of the sulfurized-phosphorized base lubricant and the same lubricant to which had been added 5% of trichlor dibenzyl was made on the Faville-Levalley machine and the former withstood a load of only 2000 pounds whereas the latter withstood a load of 4200 pounds. 60 When 8 to 10% of trichlor dibenzyl was added, the material withstood a load of 4500 pounds on the Faville-Levalley machine, which is the maximum for that machine. The E. P. characteristics of the sulfurized-phosphorized base lubricant, as determined by the Timken machine, is not appreciably altered by addition of the halogen compound. The addition of the halogenated compound, while greatly increasing the film strength and E. P. characteristics of the lubricant, had no detrimental effect thereon. Corrosion tests made in the presence of water indicate that as much as 10% of the halogenated compound may be introduced into the lubricant without rendering it corrosive.

65 The sulfurized-phosphorized base lubricant to

which 7% of trichlor dibenzyl had been added, was placed in the differential of a new automobile and the gears were checked after 1015 miles and at the end of 3638 miles. The original backlash in the gears was .006 inch. At the end of 1015 miles, the backlash was .007 inch, and the backlash at the end of 3638 miles was also .007 inch, thus indicating that the rear end "ironed" itself out within the first thousand miles and that no further measurable wear took place during the next 2600 miles. This is typical performance for a high grade extreme pressure lubricant.

Although I do not wish to be limited to the addition of any particular amount of the halogenated compound to the lubricant, I prefer to use from 3 to 10% in connection with lubricants to be used where E. P. characteristics are important. Where the compound is added to improve the oiliness and film strength, as for example, in motor oil, the amount added may range from a fraction of 1% to approximately 5%. The upper limit of 10% has been fixed only because with the methods of testing now available, it has been found that maximum results can be obtained by adding this amount. There is no reason, however, why quantities in excess of 10% may not be used.

Although I have tried chlorinated diphenyl methane in which the chlorine is linked to the carbon in the methyl radical, I have found this compound is unstable and therefore unsuitable for use.

Instead of adding the halogenated compound directly to the oil, it may be separately fed into the particular mechanism to be lubricated and mixed in situ with the lubricating oil.

What I claim is:

1. A lubricant comprising a mineral lubricating oil and a compound of the type



in which the hydrogen in the benzene rings is halogen substituted or unsubstituted, C is an aliphatic radical having any number (n) of carbon atoms in excess of one, and a halogen is united to aliphatic carbon.

2. A lubricant in accordance with claim 1 in which C is an aliphatic hydrocarbon radical.

3. A lubricant comprising mineral lubricating oil and halogenated symmetrical dixenyl butane in which a halogen is united to carbon in the aliphatic chain.

4. A lubricant in accordance with claim 3 in which the halogen is chlorine.

5. A lubricant in accordance with claim 1 and containing sulfurized and phosphorized fatty oil.

6. A lubricant in accordance with claim 3 and containing sulfurized and phosphorized fatty oil.

7. A lubricant comprising mineral lubricating oil and chlorinated 1-4 dixenyl butane in which chlorine is united to carbon in the aliphatic chain.

5 8. A lubricant comprising a major portion of mineral oil and a minor portion of a halogenated compound of the type R—C<sub>n</sub>—R' in which R and R' are non-acidic stable carbocyclic radicals, C is a straight aliphatic chain having any number (n) of carbon atoms in excess of one, and halogen is linked to carbon in the aliphatic chain.

10 9. A lubricant in accordance with claim 8 containing a minor proportion of sulfurized and phosphorized fatty body.

15 10. A lubricant in accordance with claim 8 in which R and R' are aryl radicals.

11. A lubricant comprising a major portion of mineral lubricating oil and a minor portion of halogenated dibenzyl.

20 12. A lubricant comprising a major portion of mineral lubricating oil and a minor portion of chlorinated dibenzyl.

25 13. A lubricant comprising a major portion of mineral lubricating oil and a minor portion of tetrachlor dibenzyl.

14. A lubricant comprising a major portion of mineral lubricating oil and a minor portion of halogenated compound of the type



where R and R' represent non-acidic, stable carbocyclic radicals and CH represents any aliphatic hydrocarbon radical having halogen united to the carbon in said last-mentioned radical.

15. A lubricant in accordance with claim 14 in which R and R' are non-acidic, stable aromatic nuclei.

40 16. A lubricant comprising a major portion of mineral lubricating oil and a minor portion of a compound of the type R—C<sub>(n)</sub>—R' in which R and R' are non-acidic, stable aryl radicals, C is an aliphatic hydrocarbon chain having any number (n) of carbon atoms in excess of one and a halogen is linked to carbon in the aliphatic chain.

45 17. A lubricant in accordance with claim 14 in which R and R' are non-acidic, stable aromatic nuclei and which lubricant contains sulfurized and phosphorized fatty oil.

18. A lubricant comprising mineral lubricating oil and halogenated symmetrical diphenyl diethyl ether in which halogen is united to carbon in the aliphatic chain.

55 19. A lubricant in accordance with claim 18 in which the halogen is chlorine.

WILLIAM A. WHITTIER.